

W. E. GREENAWALT,  
ELECTROLYTIC APPARATUS.  
APPLICATION FILED JAN. 11, 1912.

1,144,538.

Patented June 29, 1915.



Fig.



Fig 2



Fig 3



FIG 5

*WITNESSES:*

Thomas G Hughes  
Henry F. Bellows

*INVENTOR.*

INVENTOR.  
William Greenawalt.



# UNITED STATES PATENT OFFICE.

WILLIAM E. GREENAWALT, OF DENVER, COLORADO.

## ELECTROLYTIC APPARATUS.

1,144,538.

Specification of Letters Patent. Patented June 29, 1915.

Application filed January 11, 1912. Serial No. 670,637.

*To all whom it may concern:*

Be it known that I, WILLIAM E. GREENAWALT, a citizen of the United States, residing in Denver, in the county of Denver and State of Colorado, have invented certain new and useful Improvements in Electrolytic Apparatus.

It has for its object the attainment of higher anode and cathode efficiencies and other essential advantages which are specifically pointed out in the specification.

It is well known that in electrolysis, especially with reasonably high current densities, the electrolyte in immediate contact with the electrodes may become impoverished, and deleterious results, such as decreased efficiency and inferior deposits, are sure to follow. It has been known ever since the early experiments with electrolytic processes, that rapid changing of the electrolyte in contact with the electrodes, materially diminishes these difficulties by bringing fresh ions in contact with the electrodes at a rate corresponding with the intensity of the current.

The rapid changing of the electrolyte in contact with the electrodes may be effected by agitating the electrolyte, or, by what amounts to essentially the same thing, moving the electrodes through the electrolyte. In either case the results depend largely on the method of effectively carrying it out. The difficulty is increased if a diaphragm separates the anolyte from the catholyte.

In electrolyzing halogen solutions, in a diaphragm cell, as for example a solution of cuprous chlorid, copper is deposited at the cathode and chlorin is released at the anode. Usually, except for exceedingly small current densities, the chlorin is given off in the uncombined state, since the evolution of chlorin is more rapid than the rate of combination, due largely to impoverishment of the anolyte in contact with the anodes. For the same reason the chlorin is not dissolved in the anolyte. If the anolyte contains cuprous chlorid, ferrous chlorid, sulfur dioxid, or other reagent capable of being oxidized or changed from the univalent to the bivalent condition, the chemical combination with the chlorin is not ordinarily effective because these ions are not brought in contact with the chlorin liberated at the anode, at the same rate at which the chlorin is released. This difficulty is largely overcome by the present invention.

Referring to the accompanying drawing,

Figure 1 represents a cross section of the apparatus and Fig. 2 the corresponding plan. In these figures, one electrode is represented as being stationary or moved with a reciprocal motion, while the other electrodes are made to revolve rapidly, each on its own vertical axis. This is the preferred arrangement for some solutions. Fig. 3 shows a modification of Fig. 1, in which all the electrodes revolve each about its own vertical axis. This arrangement is preferred in other cases. Fig. 4 shows a detail section of the electrode and preferred method of suspending and revolving it, and Fig. 5, the corresponding plan.

In the figures, 1 represents an electrolytic tank, taken as a whole, 2 the cylindrical anodes revolving each about its own axis, and 3, Figs. 1 and 2, a cathode mounted on rollers 16, so that its position may be readily changed by the reciprocating mechanism 17 to insure a more uniform deposit of metal being deposited. In Fig. 3, 3' represents a revolving cathode in all respects similar to the corresponding revolving anodes. It will be understood that it is immaterial which is made the anode and which the cathode; that will depend upon the electrolyte and the results desired. The cylindrical rods 2, composing the anode as a whole, are suspended on a steel shaft 4, passing up through the frame 5 and 5', and suspended on ball bearings 6. The socket for the ball bearing is mounted on, and fastened to the frame, by means of the bolts 7, which also serves for the stationary electrical connections.

8 is a pulley fastened to each cylindrical rod and 9 a drive, such as a rope or belt, by means of which the cylindrical electrode rod 95 is made to revolve about its own vertical axis at any rate of speed desired.

In the plan, Fig. 2, are shown the electrode rods arranged in consecutive series, to form a composite electrode, acting as a whole. From this it will be seen that while the electrode as a whole, remain stationary, the individual rods composing the electrode, may be in rapid motion, and thus bring fresh electrolyte in contact with the electrodes, at any rate of speed desired.

In Fig. 2 is shown the preferred method of rotating the rods, in which the driver, which may be an endless rope or belt, passes around the driving pulley 10, then makes a half turn around the first electrode rod pulley, and so on in a sinuous line to the end of

the series for that composite electrode; the rope then passes over to the other side and similarly drives the other rods and returns again to the original driving pulley 10. It will be seen that adjacent rods rotate in opposite directions, while alternate rods rotate in the same direction. The driving pulley 10 is mounted on a sliding base, so that the driving rope may at all times be kept sufficiently taut. 12 is a diaphragm separating the anolyte from the catholyte, when necessary or desirable. For some work it may be dispensed with. In some cases it may simply be a coarsely woven material to prevent any disintegrated anode material from getting to the deposited cathode metal.

In operating the apparatus, say, in electrolyzing a cuprous chlorid solution obtained from leaching copper ores, in which it is desired to deposit the copper and regenerate the solvent, the electrolyte is introduced into the cathode compartment 14. If the diaphragms are permeable the electrolyzed cathode solution may pass through and become the anolyte; or a separate anolyte may flow through the anode compartment 15, if a dense diaphragm is used. The mechanism is then started, and the current turned on. Each anode revolves about its own vertical axis, but the combined revolving rods act as a composite whole so far as the electrolysis and diaphragm are concerned. Revolving rods could also be introduced into the cathode compartment, exactly similar to those in the anode compartment, but experience has shown that revolving cathodes in the electrolysis of copper chlorid solutions appear to be more harmful than beneficial, especially if the rotation be rapid. Provision is therefore only made, in this case, to move the cathode back and forth at intervals so as to assure a more uniform deposit, owing to the unequal distribution of the current due to the cylindrical rods. The anode rods, which for chlorid solutions, would be carbon, are easily and rapidly rotated, and once set in motion, it is only necessary to overcome the friction, due principally to the electrolyte. Copper is deposited on the cathode, and chlorin released at the anode, and were it not for the rotation of the carbon rods, much, in fact most, of the chlorin would be given off as free gas, because it would be impossible to rapidly absorb it in the electrolyte. The rotating rods bring the chlorin in contact with the electrolyte as rapidly as it is released, with the result that the ferrous chlorid in the solution is converted into the ferric chlorid, the cuprous chlorid into the cupric chlorid, and if sulfur dioxid is used as a depolarizer it will be effectively converted into sulfuric and hydrochloric acids; at the same time free chlorin may be absorbed by the electrolyte when the sulfur

dioxid has been converted into acid and the univalent compounds converted to the bivalent condition, and thus the electrolyte is more thoroughly and more effectively regenerated. These reactions, so effectively carried out, also materially reduce the necessary electromotive force required for the electrolytic decomposition. If the electrolyte were a sulfate solution, then the anodes would be likely to be composed of lead. If lead is used as the anode in the electrolysis of sulfate solutions, the lead, under ordinary conditions is rapidly peroxidized and the peroxid accumulating on the face of the anodes increases the resistance and decreases the efficiency. With the revolving anode rods the peroxid is detached about as rapidly as formed, and the rate of oxidation is diminished. In the electrolysis of copper sulfate solutions it is also desirable to have revolving cathodes similar to the revolving anodes; this insures a regeline and pure deposit of copper and a high electrical efficiency for both the anode and cathode. In other cases a stationary anode and a revolving cathode may be desired, in which case the operation would be the reverse of that described for the electrolysis of cuprous chlorin. Again, if both anode and cathode are made to rotate, it is immaterial which is made the anode and which the cathode.

The invention also finds a use in the electrolysis of substances like copper matte, in which case the matte would compose the anode, and both anode and cathode made to rotate; the anode would be rotated to facilitate the removal of the impurities such as sulfur, and to assure a uniform diminution, and the cathode to get a pure and regeline deposit. The diaphragm would act more as a filter to keep the impurities from the deposited copper.

The invention is also applicable to general refining work, and insures the equal solution of all parts of the soluble anode, with the removal of the impurities, and even deposition on the cathode. In such cases the diaphragm again would act more as a filter to keep the impurities in suspension in the anolyte from getting to the cathode compartment and on the metal deposited. Or in some cases, the diaphragm may be dispensed with entirely, especially if the rate of rotation is comparatively slow. It is well known that in depositing copper, say from a sulfate solution as the electrolyte, as the solution becomes impoverished in copper, the efficiency grows less, and the last small percentage is difficult to extract. With the rotating rods composing the electrodes an enormous amount of solution comes in direct contact with the cathode, and this, in effect, is equivalent to a more concentrated electrolyte, so that the solution may be entirely depleted of its copper con-

tent, without any perceptible diminution of efficiency and still obtain a reguline deposit. In some metallurgical work, as for example in the hydrometallurgical methods of extracting copper from its ores, it frequently becomes necessary to remove the copper from very dilute solutions. Hitherto this has been done with iron because electrolytic methods were too inefficient. With the present

5 invention this difficulty is removed owing to the enormous amount of solution brought in contact with the cathode, and the small expense of rotating the cathode rods.

10 15 The invention also finds use in the deposition and regeneration of cyanid solutions in the metallurgy of gold and silver. It finds use in the electrodeposition of zinc and of other metals. It also finds use in

20 other electrolytic arts, but the apparatus has been sufficiently described to make its purpose clear, and its application to any particular process or use may be readily understood and determined. The elec-

25 25 trodes are suspended and attached to the frame consisting of the longitudinal pieces 5 and the cross pieces 5<sup>a</sup>, so that the entire frame and electrodes may be lifted out of the electrolyte tank for inspection or trans-

30 ference to another tank.

Up to the present time it has been an insurmountable difficulty to adapt diaphragms to rotating electrodes. I am not aware that this has ever been accomplished 35 on a practical working basis, and except for small porous pots made of clay or earthenware, it is practically impossible to construct a working diaphragm on curved lines. It is claimed for this invention that 40 all electrolytic apparatus designed on this basis retain all the simple features of the simplest diaphragms, while realizing all the advantages of moving electrodes or of agitating the electrolyte.

45 I am aware that cathodes, and both soluble and insoluble anodes have been rotated around a vertical axis in electrolytic work, but

What I claim specifically, is:

50 1. In electrolytic apparatus the combination of an electrolyte tank; a straight diaphragm separating the anode from the cathode compartment; a composite electrode composed of a series of cylindrical 55 rods arranged in a straight line and each

rotating about its own vertical axis, and means for rotating the cylindrical rods of the electrode with a common driver.

2. In electrolytic apparatus the combination of a tank containing the electrolyte; a straight diaphragm dividing the tank into anode and cathode compartments; a moving cathode, and a composite anode composed of cylindrical rods arranged in a straight line, and each revolving about its own vertical axle, and driven by a common driver.

3. In electrolytic apparatus the combination of a straight reciprocating cathode and composite anode composed of a series of suspended cylindrical rods arranged in a straight line, each revolving about its own vertical axis, and driven by a common driver.

4. In electrolytic apparatus the combination of a cathode tank; a straight diaphragm dividing the tank into anode and cathode compartments; a straight reciprocating cathode, and an anode composed of a series of cylindrical rods arranged in a straight line, each revolving about its own vertical axis, and driven by a common driver.

5. In electrolytic apparatus the combination of an electrolyte tank; a straight diaphragm separating the tank into anode and cathode compartments; moving cathode in the cathode compartment, and composite anodes on both sides of the cathode composed of cylindrical rods arranged in a straight line, each rotating about its own vertical axis, and driven by a common driver.

6. In electrolytic apparatus the combination of an electrolyte tank; a straight diaphragm dividing the tank into anode and cathode compartments; a frame over said tank; cylindrical rods arranged in a straight line in consecutive series suspended from the frame and forming a composite electrode; revolvably mounted bearings from which the rods are suspended; means for rotating the rods each about its own vertical axis with a common driver, and electrical connections through the stationary socket of the bearings to the revolving electrodes.

WILLIAM E. GREENAWALT.

Witnesses:

THOMAS C. HUGHES,  
HENRY F. SELLERS.